

# UNITED STATES PATENT OFFICE.

JEFFERSON L. FULTON AND JULIUS BRACE, OF COVINGTON, KENTUCKY.

## IMPROVEMENT IN BITUMINOUS-ROCK PAVEMENT.

*Specification forming part of Letters Patent No. 103,168, dated May 17, 1870.*

*To all whom it may concern:*

Be it known that we, JEFFERSON L. FULTON and JULIUS BRACE, of Covington, county of Kenton, State of Kentucky, have invented a certain Process for Preparing Paving and Roofing Materials, of which the following is a specification:

The nature of our invention consists in laying a pavement composed of crushed bituminous limestone with finely-pulverized material and bitumen added to form a base for a strong cement, the whole, when laid, forming a strong, hard, durable artificial rock or concrete pavement.

To enable others to prepare the same, we will proceed to describe the process and articles used by us which we deem to be the best, though both may be varied in many ways without changing their character.

The necessary elements used in the process are bituminous limestone, which contains from eight to fifteen per cent. of bituminous matter infused into the rock. This is a natural product, and found in the city of Chicago, Illinois, in a quarry situate near the intersection of Western and Grand avenues. This limestone is crushed and used with artificial asphalt or natural bitumen, (with "dead-oil" to set or soften the asphalt,) pure dry clay or finely-pulverized stone, or other similar substances, to give body to the cement. Sharp sand or broken stone or gravel may be used to add to the durability, but it is not necessary with ordinary rock-bitumen.

If foreign sand or stone be used, not over twelve per cent. should be employed.

Natural rock-bitumen, which does not contain bituminous substances enough for the cementing properties required, will receive and take up artificial asphalt, if used with dead-oil, whose specific gravity is greater than water and its vaporizing-point not less than 230° Fahrenheit, and will form an artificial compound much more durable than any combination of mineral substances and asphalts hitherto used.

We deem the following proportions the best adapted for ordinary pavements, though they may be varied as the pavement is required to be cheap or durable, elastic or hard:

Rock bituminous limestone, one hundred and

fifty parts; pure dry clay, twenty-five parts; bitumen, either natural or artificial, twenty-five parts; with two parts dead-oil or hydrocarbon oil of the gravity above named; and twenty-five parts sand or broken stone.

Take the bituminous limestone, and powder or crush in any ordinary mill. One-third of the amount should be well pulverized. The remainder may be in pieces not larger than one-half inch in diameter.

The quality of the rock should then be tested, to ascertain the amount of bituminous matter contained in it, to ascertain the amount of asphalt and mineral hydrocarbon oil to be added.

The rock-bitumen should contain from eight to fifteen per cent. of bituminous matter, and enough asphalt should be added to make the entire mass from fifteen to twenty per cent. bituminous. This test may be made by exhaustive distillation, or by dissolving in naphtha or light hydrocarbon oil, in which the bitumen in the rock is easily soluble.

The crushed and pulverized rock should then be subjected to a slow process of heat, ranging from 200° to 230° Fahrenheit, and thoroughly stirred till the bitumen and rock are sufficiently softened to coalesce, and until the bituminous matter be added, which should be ten parts asphalt and one part dead-oil. Twenty-five parts of pure dried clay, chalk, or fine pulverized rock are then added. The whole mass should be thoroughly stirred during the entire process of heating. Twenty-five parts of fine sharp sand or broken stone may be added without materially affecting the tenacity of the cement, while it adds to its durability. The whole mass is continued at a temperature of not more than 230° Fahrenheit, and stirred or agitated until the compound is thoroughly mixed, when it may be put down into pavements.

If it is desired to be prepared for putting down into pavements or making roofs at a future time the pulverized clay and sand should not be added, but the compound can be run into cakes, and easily transported to any desired place. When it is desired to use the material, it should be again heated and melted, the clay and sand added, as before described, and put down while hot, in the manner described.

To have the cement sufficiently strong to bind and unite all the elements, it should contain in all from fifteen to twenty per cent. of bituminous substances, and the asphalt-oil is added to give it the required tenacity. The clay or pulverized rock forms the body of the cement, which coalesces with and forms a complete chemical combination with the bituminous substances, natural and artificial. The clay also acts as a non-conducting agent in repelling the rays of the sun. The natural porosity of the rock, with the clay and cement, render the material elastic. The more clay and pitch used, the more elastic will be the compound. When combined in the manner described, the material, when cold, forms an artificial bituminous stone or concrete unlike any other material yet used.

After the ingredients are all properly mixed and combined, the heat is continued till the natural bitumen of the rock and the asphalt are all thoroughly incorporated with each other and with the mineral atoms, which must be thoroughly impregnated to form a complete combination with each other.

The composition is taken while hot and laid upon the street or sidewalk, which must first be thoroughly prepared, and should be treated to gravel sufficiently to take away all moisture from the surface, and thoroughly packed with any material that will form a solid dry base for the pavement. The composition is then

laid down while hot, and tamped or rolled as it is laid down till the particles are all thoroughly united. When cold, it becomes perfectly hard, with sufficient elasticity to prevent breaking.

For street-pavements, with a proper base, three inches of the compound are sufficient to make a street for the heaviest wear. For sidewalk, one inch of the compound is sufficient.

Stone of similar nature and utilized to similar process is found near Eaton, Preble county, Ohio, and in various parts of Kentucky. These products differ from the Seyssel rock-bitumen, which dissolves or crumbles into dust at about 212° Fahrenheit, while the American bitumen stone will not dissolve without heat so great that the bituminous matter would be consumed before dissolving or "crumbing."

Having thus described our invention, what we claim as new, and desire to secure by Letters Patent, is—

A pavement, composed substantially of bituminous rock, asphalt, and fire-clay, or other similar substance, prepared and laid down as herein set forth.

JEFFERSON L. FULTON.  
JULIUS BRACE.

Witnesses:

E. E. WOOD,  
HERMAN MERRILL.